

Dec. 22, 1931.

A. R. BRADEN

1,837,523

## ART OF MAKING CLICKING DIES

Filed Jan. 7, 1928

2 Sheets-Sheet 1



## INVENTOR.

Albert R. Braden  
By his Attorney,  
Nelson W. Howard

Dec. 22, 1931.

A. R. BRADEN

1,837,523

## ART OF MAKING CLICKING DIES

Filed Jan. 7, 1928

2 Sheets-Sheet 2



Fig. 3.



Fig. 4.



*Albert H. Braden  
By his Attorney  
Nelson M. Howard*

## UNITED STATES PATENT OFFICE

ALBERT R. BRADEN, OF BEVERLY, MASSACHUSETTS, ASSIGNOR TO UNITED SHOE MACHINERY CORPORATION, OF PATERSON, NEW JERSEY, A CORPORATION OF NEW JERSEY

## ART OF MAKING CLICKING DIES

Application filed January 7, 1928. Serial No. 245,221.

My invention relates to the making of clicking dies, such as are employed for cutting out parts of shoes, it involving a method of producing these dies. The improved die-stock 5 preferably employed in performing this method is made the subject of a divisional application Serial No. 433,450, filed in the United States Patent Office on March 5, 1930.

The stock from which clicking dies are customarily manufactured consists of strip-steel tapered in cross-section, the opposite sides diverging from an edge which is to furnish the cutting portion to a thicker edge to which pressure is applied during the cutting operation. In rolling the stock, the heat used to condition the metal burns out the carbon over the surface, forming an outer layer or skin which cannot be properly tempered. Consequently, in making dies from the strip, the decarbonized scale near the cutting-edge portion must be ground away to expose the steel having the full carbon-content. On the other hand, the decarbonized portion is tough and resistive to pressure, so it is desired that the exterior of the stock toward the thicker edge, or all that need not be tempered, shall remain undisturbed to gain the benefit of the strength of this surface-layer. To maintain consistently the correct relation of the ground and unground areas, with the usual practice followed in manufacture, is extremely difficult. When the removal of the scale is done in the strip, the stock is not straight, but contains waves, which may sometimes be quite abrupt. The result of such changes of direction is that, as the workman guides the strip before the grinding wheel, the departure of its side from a straight line may cause the decarbonized skin to be taken off below the area to be tempered, even completely to the pressure-receiving edge; or opposite curvature of the stock may lead to the removal of too little material, the decarbonized surface remaining close to the cutting portion. For the reasons already stated, the resulting die, in the first instance, will not be as durable as it might, and, in the second, there will be soft spots in the cutting edge. It is an object of this invention to provide for the production of clicking dies which will have the full benefit of

the strength of the decarbonized material where this produces no harmful effect, yet will be substantially free from it where it will interfere with the temper of the cutting edge.

For the attainment of this object, this invention provides a method of die-making in which a gage-line extending longitudinally of a strip of stock, furnishes a guide for the workman in the removal of material near the cutting-edge portion. The gage-line is provided by a unitary projection from the stock, to which the grinding or other material-removing operation is substantially confined. The projection thus performs the double function of creating a guide and giving a body of material within which there will be an opportunity for cleaning the area to be tempered without overrunning upon the portion over which the retention of the surface-strength is desired. This increased thickness at the cutting edge also strengthens it. In completing the die from the stock treated as just outlined, it may be bent to form with the surface from which the decarbonized material has been removed at the inside, and then such material removed from the opposite side. After this, it is tempered and sharpened by grinding the outside. With the strip made up in die-form, the short lengths, changing in direction according to some definite plan, are much easier to follow in the removal of the decarbonized skin than in the strip-form. While not always necessary, the projection may be provided upon both sides of the stock, so there is a double guiding means and body of material within which to work safely.

Means for performing the steps of my improved method and the die-stock operated upon are illustrated in the accompanying drawings, in which

Fig. 1 is a perspective view of a mill by which the stock may be rolled;

Fig. 2 is a similar view of a grinding apparatus for removing the decarbonized skin from one side of the strip of die-stock;

Fig. 3, a perspective view of a bending device employed in forming the die;

Fig. 4, a like view of a grinding apparatus by which the decarbonized portion may be

removed from the exterior of the formed die;

Fig. 5, a view showing, in perspective, a grinding apparatus by which the die may be sharpened;

Fig. 6, a perspective view of die-stock having projections from its opposite sides;

Fig. 7, a similar view showing the stock after it has been operated upon by the apparatus of Fig. 2; and

Fig. 8, a view corresponding to Fig. 6, in which appears another form of die-stock.

A mill M, partially shown in Fig. 1, has rolls 10, 10, of which two of a vertical series of three are illustrated. These rolls are adapted to produce, by steps successively performed, as by sections 12, 12; 13, 13; and 14, 14, upon a heated metal bar b, a strip of clicking-die stock. The roll-sections 12 give to the bar a preliminary form, the sections 13 an intermediate form, and the sections 14 the final form B. The stock B, shown most clearly in Fig. 6, has a portion c, in which the cutting edge of the clicking die is to be produced, and at its opposite edge a thicker portion d, to which, in the finished die, cutting pressure is applied. The opposite side walls of the strip diverge gradually toward the thick edge, except that, near the cutting-edge portion, there is a projection, in the present instance one being shown at each side. Each projection is angular, having, at its outer side, two walls, one e extending from the thin edge of the die to an apex f, and the other wall g extending from the apex to a line h, where the wall g meets the normally inclined wall m of the strip. Both the apex-line f and the line h are substantially parallel to the opposite edges of the strip. The walls e and g form with each other an obtuse angle approaching quite closely to 180 degrees. One reason why this obtuse angle is important is that, as the wall g is made more nearly perpendicular to the wall m, it becomes increasingly difficult to roll the stock without causing the portion at the apex f to be broken or irregular, the depth of the fractures being sometimes such as to make the stock unsuitable for the formation of the cutting edge.

In manufacturing a die from the stock B, the decarbonized surface is removed from one side of the strip at the portion c where the cutting edge is to be produced. A grinding apparatus G for this purpose appears in Fig. 2. Upon a base 16 is mounted a slide 17 having, pivoted on it, a tilting table 18, the angle of which may be varied by a screw 20. Studs 22 and 24, having their peripheries inclined oppositely to the wall of the strip, guide it to be ground as it is moved by the operator across an abrasive wheel 26. The stud 24 is shown as under the influence of a spring 28, by which the strip B is forced against the wheel, and the grinding relation may be further varied by the movement of the slide 17

upon its base. As the operator advances the stock, he watches the lower edge i (Fig. 7) of the bright area k, created by the wheel 26 as it removes the dark decarbonized scale, comparing its relation to the gage-line h of the stock-projection. If, on account of curvature or other irregularities of the strip, there is a material departure from the edge i of the gage-line, the stock is moved slightly toward or from the wheel by shifting the slide. In this way, the ground area may be caused to comprehend the decarbonized portion in proximity to the cutting edge, and thus place this edge in condition for tempering, while at the same time disturbance is avoided of the tough skin at m, near the pressure-receiving edge d, where its strength is desired. It should be noted particularly that, since the grinding takes place within the projection furnished by the angular walls e and g, and since it is not necessary to wholly remove this projection to complete the clearing-off of the scale at the cutting-edge portion, there may be considerable variations in the form of the strip, without causing the ground area k to overrun upon the area m. That is, there is in the projection, beyond the normal taper of the clicking-die stock, a body of material within which variations in the depth of grinding may occur without evil effect.

The side of the stock which has been ground as just described is to be at the inside of the die, and the edge at n is brought into conformity with a templet T (Fig. 3) by bending, as with hand-tools, aided by such a device as a press P having a fixed abutment 30 and a movable member 32. Having been formed to the outline of the templet, the ends of the piece are welded together, giving the die D.

The decarbonized skin is now to be removed at the outside of the die to produce the clean area adjacent the cutting edge, as already done at the inside while in strip-form. For this purpose, a simple grinding apparatus H may be utilized, this having a tilting table 34 to support the die, said table being adjustable as to angle by a screw 36. With the table, an abrasive wheel 38 cooperates. In this operation, when employing the stock B having a projection at both sides, the procedure may be similar to that described in the preceding step, and the result the same. The operator shifts the die upon the table, increasing or decreasing its pressure against the wheel 38, as may be necessary to remove the proper amount of material and bring the line i of the ground area in the correct relation to the gage-line h. It may be found that, because the work operated upon is in short lengths without unexpected changes in form, or when the workmen are skillful, it will be unnecessary to employ the projection with its gage-line at the outside

of the stock. In this case, the stock may take the form appearing at C in Fig. 8. One side, as that to be acted upon before forming, is as in the stock B of Fig. 6, while the other, at  $\sigma$ , 5 has a gradual taper from the cutting-edge portion  $c$  to the pressure-receiving portion  $d$ . This latter corresponds to the well-known cross-sectional outline of clicking-die stock.

10 Having been thus formed to the templet and prepared for tempering by the removal of the decarbonized skin from both sides, such tempering is effected in the customary manner, and finally the die is sharpened, as 15 by a grinding apparatus I, in which a table 40 supports the die and presents it to a wheel 42 rotatable about an inclined axis. This completes the more essential operations of die-production. After sharpening the die, 20 its cutting edge is backed by a greater thickness of metal than in the usual form of die, because the added thickness between the sides of the stock along the line  $f$  is not all ground away. Increased strength at the cutting edge 25 is therefore obtained.

By employing the method of this invention, dies may be manufactured having a high degree of uniformity with respect to the ground area, from which the decarbonized 30 portion has been completely removed for tempering the cutting edge, and the unground area, upon which said material is retained because of its strength. These results are possible when the workmen have 35 no more than ordinary skill.

Having described my invention, what I claim as new and desire to secure by Letters Patent of the United States is:

1. The method of making clicking dies 40 from a strip of stock having a longitudinally extending projection furnishing a gage-line, which consists in grinding under the guidance of the gage-line material substantially confined to the projection.

45 2. The method of making clicking dies from a strip of stock having a longitudinally extending projection furnishing a gage-line, which consists in grinding under the guidance of the gage-line material substantially 50 confined to the projection, and forming the ground strip to complete the die.

3. The method of making clicking dies, which consists in forming a strip of die-stock with a unitary projection extending 55 along the strip near the cutting-edge portion, and removing material for the production of the cutting edge, such removed material being substantially confined to the single projection at the side of the strip thus 60 operated upon.

4. The method of making clicking dies from stock having a decarbonized coating, which consists in forming a strip of die-stock with a projection extending along the strip 65 near the cutting-edge portion, removing de-

carbonized material from one side of the strip by grinding the projection, forming the strip to the outline of a clicking die with the surface from which the decarbonized material is removed at the inside, and grinding 70 the outside of the die.

5. The method of making clicking dies, which consist in rolling a strip of die-stock with a projection extending along the strip 75 near the cutting-edge portion, grinding the projection to remove decarbonized material from one side of the cutting-edge portion, bending the strip to the form of a die with the ground portion at the inside, grinding the outside of the die to complete the removal 80 of decarbonized material from the cutting-edge portion, and tempering and sharpening the cutting edge.

5. The method of making clicking dies, which consist in rolling a strip of die-stock 85 with a unitary projection along each side of the strip substantially parallel to the cutting-edge portion, and removing stock for the production of the cutting edge, such material removed being substantially confined 90 to the projections.

7. The method of making clicking dies from stock having a decarbonized coating 95 which consists in forming a strip of die-stock with projections along opposite sides of the strip near the cutting-edge portion, grinding one of the projections to remove decarbonized material at one side of the cutting-edge portion, bending the strip to the form of a die with the ground portion at the inside, grinding the outer projection to complete the removal of the decarbonized material from the cutting-edge portion, and tempering and sharpening the cutting edge. 100

In testimony whereof I have signed my 105 name to this specification.

ALBERT R. BRADEN.

110

115

120

125

130